

July 12, 1932.

F. H. SCHAVOIR

1,867,103

GOLF CLUB HEAD AND PROCESS OF MAKING THE SAME

Filed Nov. 23, 1927

Fig. 1.



Fig. 2.



Fig. 3.



Inventor  
F. H. Schavoir

By

Robert B. Rock

Attorneys

## UNITED STATES PATENT OFFICE

FREDERICK H. SCHAVOIR, OF STAMFORD, CONNECTICUT, ASSIGNOR TO SCHAVOLITE GOLF CORPORATION, OF NEW YORK, N. Y.

## GOLF CLUB HEAD AND PROCESS OF MAKING THE SAME

Application filed November 23, 1927. Serial No. 235,225.

In the manufacture of golf clubs, particularly those known as drivers, brassies and spoons, it has been universally considered necessary to employ a head made of wood because of the known characteristics of such material for affording the desired resilience, durability and finish in clubs of this type; but in view of the many difficulties experienced in the manufacture, in respect to the attainment of a proper balance, concentration of weight, and duplication of patterns—all more or less influenced by the seasonings of and natural differences in the species of the woods, their tendency to shrink, etc.—many efforts have been made to find a substitute which would enhance the qualities possessed by the wood and at the same time facilitate the accuracy and consistency of manufacture.

In the formation of these club heads it is necessary for each one to be individually shaped by a highly skilled worker who carefully trims the body away by degrees until according to his "feel" it has the proper weight and balance so that actually the quality of the club and the accuracy which may accompany its use depend primarily upon the degree of skill of the particular artisan. However, no two workmen may have the exact amount of skill or the same grade of material from which to fashion the club head, and hence it is practically impossible to duplicate or produce standardized or consistently accurate constructions of clubs.

To overcome the deficiencies of the materials, many expedients have been resorted to, among which may be mentioned the application of metal, ivory and other weight imparting materials to the club head which not only add to the expense of manufacture but harmfully affect the "control" in the use of the club because unless the impact with the ball occurs at the proper spot of the striking face in relation to the concentration of the weight, the tendency is to turn or twist, resulting in undesired "slicing" and "hooking".

It has even been proposed to form the heads completely of metal or mostly of metal, but a considerable amount of resiliency is sacrificed in so doing.

To overcome the foregoing difficulties it

has been my aim to provide a molded club head of resilient material, such as vulcanized rubber which has been so treated in the vulcanizing process as to possess that degree of hardness required for obtaining the maximum distance of flight of the ball and yet insure that durability in use which is necessary. My invention therefore resides in the provision of a new article of manufacture in the form of a molded, vulcanized rubber club head and a novel process of producing the article in such a manner that the exposed surface of the head possesses the necessary degree of hardness, which hardness gradually decreases toward the center, whereby the driving surface is backed by a resilient or elastic mass to produce the acceleration in the drive which will give the greatest distance in flight.

Before proceeding with the description of my improvements, it is to be noted that I am aware of the fact that it has been heretofore proposed to provide rubber striking faces for golf clubs or rubber inlays or inserts, but these are very unsatisfactory because of the different shrinkage characteristics of the materials, the difficulty of permanent attachment, and the effects of moisture upon the component parts of the head, to say nothing of the increased labor costs. Attempts to overcome these problems have been made by using phenolic condensation products which may be molded. This substance, however, is unsuitable for the purposes because it is impossible to control the hardening and because of its tendency to brittleness and fracture, requiring the use of embedded reinforcing means which render it extremely difficult to produce a well balanced head.

In carrying out the process which constitutes an embodiment of this invention, the following ingredients may be employed in about the proportions which are specified: 32 parts rubber, 50 parts ground hard rubber dust, and 18 parts sulphur, together with a small amount of a known accelerator such as diphenol-guanadine.

It is to be specifically understood that the foregoing formula is given as an exemplification, and that the same may be modified so as to change the ingredients or proportions

where different ingredients or fillers are used, and I therefore do not wish to be limited in this respect. For example, if the rubber content is increased, necessarily the sulphur would be increased and the amount of rubber dust which is employed as a filler would be reduced. These materials are mixed together in a dry state in a regular rubber working machine until the "dough" has been thoroughly conditioned. Then a suitable amount of the same is placed in a properly shaped mold of the two-part type in which the tubular bushing which forms a part of the club head is preliminarily disposed. The mold is then placed in a suitably heated press and subjected to vulcanizing heat for a period of approximately thirty minutes. The mass at the end of this first heating stage has imparted to it the desired shape but is still in a pliable condition. It is now removed from the mold and subjected to open heat at about 280° F. for a period of about three hours, depending upon the particular formula which may be employed. It is to be understood that the second stage of vulcanizing or hardening is carried to a point which is short of rendering the material brittle or frangible. The surface of the head is now ground to remove all projections and then polished on a cotton wheel in the usual manner; after which the staff is sealed or fixed in the tapered socket formed by the tubular bushing.

In carrying out the vulcanizing process, advantage is taken of this bushing to effect a transmission of the heat to the interior of the rubber mass, and by virtue of the resultant internal and external heat a body is formed in which the outer surface is relatively hard because of its direct contact with the heat, the hardness gradually decreasing toward the center. In other words, the impact receiving surface is backed by a resilient and elastic core, as above premised, and this is an important feature of my invention which gives rise to the advantageous results referred to. In order to present a comparative result I note the following tests made with a scleroscope:

A steel ball weighing 15 grams was dropped a distance of 20 centimeters onto a series of six club heads, producing a range of rebound readings from 45 to 53. This same test made with a piece of high grade wrought iron onto which the ball was dropped every one-eighth inch produced readings from 12 to 24, showing clearly the great degree of elasticity or resiliency possessed by my article.

It is of course desirable to employ a bushing of material possessing good heat conducting characteristics, such as aluminum, brass or the like, and preferably this bushing is of tubular form.

In the drawing:

Figure 1 is a side elevation of a golf club

constructed in accordance with my invention, portions being broken away and shown in section to disclose the details of construction;

Figure 2 is a top plan view; and

Figure 3 is a perspective view of the tubular bushing or shaft socket.

The vulcanized rubber body of the club head is designated by the numeral 1, and the bushing 2. It will be noted that the outer end of the tube is reamed out to provide a taper for the correspondingly formed end of the shaft, while the inner end of the bushing is flattened to prevent the passage of the rubber to the shaft socket. Preferably this bushing extends throughout the length of the club head or the major portion thereof.

By following the foregoing process a club head of the exact shape and weight desired is obtained and having the resiliency required without the tendency to split off or break. Further, no difficulty of reproduction exists once the proper form of the head is obtained and the expense of manufacture of the article is materially reduced. It is to be understood, of course, that a metal base plate may be provided for the club head and where this is desired the plate is simply formed with the necessary connecting flanges or projections and laid in the base of the mold before the rubber is introduced into the same. In the hardening of the rubber the plate becomes firmly attached to the body and requires no other fastening means. While this is of considerable importance in my product, it is deemed unnecessary to illustrate the same because it will be readily understood from the foregoing description.

Having thus described my invention, what I claim as new and desire to secure by Letters Patent of the United States is:

1. A golf club head or the like formed of homogeneous vulcanized rubber having a relatively hard impact surface backed by a resilient mass.

2. A golf club head or the like formed of molded vulcanized rubber having a relatively hard exterior and a solid non-hardened elastic interior.

3. A golf club head or the like of vulcanized rubber comprising a solid body vulcanized to a hardness gradually decreasing from the surface to the interior center.

4. A golf club head comprising a body formed of a molded relatively hard and resilient composition and having a core member of heat conducting material extending throughout the major portion of the body.

5. A golf club head comprising a solid body of molded relatively hard and non-frangible vulcanized resilient rubber having embedded therein a shaft receiving bushing extending from the heel to the toe of the body.

In testimony whereof I affix my signature.

FREDERICK H. SCHAVOIR. 130